

## UNITED STATES PATENT OFFICE

2,262,926

## FLUSHING OIL COMPOSITION

John A. Edgar and Harold A. Woods, Martinez,  
Calif., assignors to Shell Development Company,  
San Francisco, Calif., a corporation of  
Delaware

No Drawing. Application September 24, 1940,  
Serial No. 358,129

2 Claims. (Cl. 252—161)

The present invention relates to compounded flushing oils for use in internal combustion engines.

As is known, deposits of lacquer, viscous asphaltic oxidation products of oil and lacquer-bound solid particles form on piston rings, ring grooves, cylinder walls, oil lines, oil screens and crankcase walls of internal combustion engines during use. These deposits lead to piston ring sticking, interruption of oil circulation, increased oil consumption, abrasion of bearing surfaces and eventual engine destruction if not removed.

It has been the practice to attempt the removal of these undesirable engine deposits by flushing the engine with light mineral oils and/or various compounded preparations.

It is an object of the present invention to provide an improved compounded flushing oil suitable for removal of the above-described engine deposits. Further, it is an object of the instant invention to provide a single compound with a double cleansing action, i. e. both an excellent lacquer solvent and an excellent cleanser for carbon sludge deposit removal. Still further, it is an object to provide a flushing oil having a sufficiently high flash point to enable its safe use under all conditions and one which is stable under storage conditions. Other pertinent objects are to provide a flushing oil having satisfactory lubricating properties, one that is rapid and thorough in its cleansing action and at the same time non-corrosive with respect to the various metal alloys used at the present time in internal combustion engine construction. Other objects will appear in the following detailed description of the invention.

Internal combustion engines become fouled after continued operation by contamination of the lubricating oil with solid particles such as carbon, metal particles and road dust and by the gradual deterioration of the lubricating oil and subsequent formation of lacquers. Several of the more specific serious effects which will occur if engine fouling is permitted to follow its normal course are as follows:

Solid particles deposit in the ring grooves behind the piston rings, are cemented together by lacquer formation arising from lubricating oil deterioration and build up to such an extent that normal flexing of the ring is prevented; as a result, ring sticking ensues.

Solid particles entrained in an emulsion of asphaltic material, oil and water, deposit on the oil screen and in small drilled oil passages, at times completely obstructing the oil circulatory

system and in any case resulting in impaired, faulty lubrication of the various parts of the engine.

Lacquer is deposited on cylinder walls, in 5 severe cases in sufficient thickness to cause the piston rings to be imbedded therein and effecting cementation of the piston rings to the cylinder walls, resulting in piston seizure when the engine is stopped.

10 Solid matter, oxidized oil products and water form sludge deposits on the crankcase walls, in valve chambers and in other areas where there is little agitation. These deposits are particularly harmful when they obstruct penetration of 15 oil to the valve guides and similarly lubricated elements of the engine.

Lacquer deposits build up on top and bottom of piston rings and/or ring grooves, thus inhibiting normal ring flexing and eventually causing ring 20 sticking.

Other phenomena such as, for example, pre-ignition and detonation due to carbon deposition in the combustion chambers and increased oil consumption due to plugging of the slots and 25 holes of the oil control rings, among others, will inevitably result if internal combustion engines are not periodically cleaned to remove these undesirable deposits.

Since it is impractical to disassemble an engine 30 every time sludge and lacquer deposits build up to a point where their removal becomes necessary, such removal is usually attempted by utilization of cleaning agents which may be either added to or substituted for the lubricating oil normally 35 present in the engine crankcase. As had been mentioned above, it has been standard practice in the past to attempt to use light lubricating oils for this purpose; it is obvious, however, from the very nature of the fouling material that mineral 40 oil in itself is not a satisfactory solvent or cleaning agent. More recently, it has been found that superior results may be attained by using compounded flushing oils comprising essentially a solvent for the lacquer deposits encountered, a 45 detergent to loosen and/or emulsify the sludge deposits and sufficient lubricating oil to ensure safe operation during the cleansing period.

The instant invention relates to an improved compounded flushing oil of the type last described above.

The requisites of an effective flushing oil are:

1. It must be a good solvent for lacquer and resins.
2. It must have a suitable detergent action in order to carry away solid particles.

3. The flash point must be high enough to permit safe use in an engine.
4. It must not be corrosive, especially with regard to bearing metal alloys.
5. It should preferably have a relatively low viscosity (of the order of 100 S. S. U. at 100° F.).
6. It must have sufficient lubricating properties to ensure safe operation of an engine for at least short periods.
7. It should be sufficiently stable to withstand storage for long periods.

According to the present invention, a composition containing the following ingredients has been found to have all the above desirable properties: a highly aromatic hydrocarbon material having a wide boiling range such as, for example, a blend of high viscosity lubricating oil or, alternatively, a lubricating oil extract such as furfural extract, or similar aromatic extracts having a high viscosity and boiling over approximately the same range (that is, 300° F. to 500° F. or more) at 1 mm. Hg., and a highly aromatic  $\text{SO}_2$  soluble petroleum extract having a boiling range of approximately 400° F. to 600° F. such as kerosene extract; a petroleum sulphonate which is either neutral or slightly acid as a detergent; a lacquer solvent having high boiling and flush points such as diacetone alcohol; water.

A preferred composition contains the above materials in the following proportion by weight:

|                                                                    | Percent |
|--------------------------------------------------------------------|---------|
| 150 S. S. U. at 210° F. lubricating oil or lubricating oil extract | 50      |
| Kerosene extract (boiling range 410° F.-510° F.)                   | 34      |
| Sodium salt of mahogany sulfonic acid                              | 10      |
| Diacetone alcohol                                                  | 5       |
| Water                                                              | 1       |

The above flushing oil composition has a viscosity of 100 S. S. U. at 100° F. The flash point is above 150° F. as determined by the Pensky-Martens closed cup method (A. S. T. M. designation: D93). There is no phase separation upon storage and no appreciable semi-solid bottom deposits after subjection to four days storage at 40° F., five hours storage at 30° F. or one-half hour of centrifuging under 1000 g. force.

The relative quantities of the various constituents set out in the above preferred formula may be varied within certain limits without deleteriously affecting the beneficial effects and desirable properties thereof to an undue degree. The water content may be altered from any value less than 1% to a maximum of 5%, depending largely upon the tendency for an aqueous phase to separate. The tolerance of the composition with respect to water is largely dependent upon the aromaticity of the hydrocarbon blend used. The content of diacetone alcohol may be varied from 2% to a maximum of 10%. The amount of petroleum sulphonate may vary from 5% or less to as much as 25%, although more than 15% is not normally recommended. The product commonly known to the trade as Twitchell's Base No. 262 is preferably used for this constituent, being a sodium salt of mahogany sulfonic acid plus a small amount of a stabilizing agent, such as for example cyclohexanone. The lubricating oil or lubricating oil extract and aromatic lighter extract, such as kerosene extract, taken together, may vary from 60% to 85% of the composition. It is preferable to utilize as much of the lighter aromatic extract as possible, but since the viscosity of such extracts is usually low (of the or-

der of 40 S. S. U. at 100° F.), the determining factor of the proportions of these two constituents is that the final flushing oil composition should have a viscosity of approximately 100 S. S. U. (seconds Saybolt Universal) at 100° F., and in no case appreciably less than this.

It will thus be seen that the heavier the grade of lubricating oil or lubricating oil extract used, the greater the quantity of lighter aromatic petroleum extract that may safely be utilized.

It has also been found desirable at times to provide a flushing oil concentrate, this material being diluted with a light mineral oil before use. The following has been found to be a satisfactory concentrate composition:

|                                                                 | Percent |
|-----------------------------------------------------------------|---------|
| 200-230 S. S. U. at 210° F. heavy lubricating oil               | 33      |
| Highly aromatic petroleum extract boiling in the kerosene range | 27      |
| Twitchell's Base No. 262                                        | 20      |
| Diacetone alcohol                                               | 10      |
| Water                                                           | 10      |

This composition is diluted with sufficient light lubricating oil, usually about 1:1, to produce a final blend having a viscosity of approximately 100 S. S. U. at 100° F.

The recommended procedure for cleaning an internal combustion engine with the herein described flushing compound is as follows: the crankcase is drained while the engine is hot to remove as much of the old lubricating oil present as possible; the crankcase is then filled with the instantly described flushing oil composition, the engine started and operated at a fast idling speed for one hour and the crankcase again drained; the crankcase is then filled with a light mineral flushing oil, the engine started and operated for a period sufficiently long to remove any of the flushing oil composition held up in the various parts of the engine, after which the crankcase is again drained and is then ready for its normal charge of lubricating oil.

Numerous laboratory and field tests on various engines indicate that the cleansing treatment as described above results in removing a major proportion of all sludge and lacquer deposits in the oil rings, ring grooves, oil holes, oil screen and oil lines. Lacquer deposits are completely removed in most cases from the piston skirts and other parts, carbon on the piston crowns softened and the quantity thereof reduced and most of the sludge and heavy, viscous, oxidized oil deposited on the crankcase walls is removed.

As a specific example, a test engine was first flushed with a light mineral oil, this oil being then drained and extracted with ether. A residue of 1.9 grams of insoluble solid was recovered after filtration. The same engine was then flushed with the presently described flushing oil composition, the same extraction procedure followed, and as a result another 11 grams of insoluble, solid material was recovered after filtration. The results of this test indicate that the above flushing oil composition is nearly 6 times as effective in removing undesirable engine deposits as a light mineral oil.

We claim as our invention:

1. A flushing oil composition suitable for removing sludge and lacquerous deposits from internal combustion engines comprising substantially not more than 5% by weight of water, from 2% to 10% by weight of diacetone alcohol, from 5% to 25% by weight of a sodium salt of mahogany sulfonic acid having a pH not exceed-

## Percent

|                                                                                               |    |
|-----------------------------------------------------------------------------------------------|----|
| Mineral lubricating oil having a viscosity of approximately 150 S. S. U. at 210° F.           | 50 |
| Highly aromatic liquid sulfur dioxide soluble petroleum extract boiling in the kerosene range | 34 |
| Sodium salt of mahogany sulfonic acid                                                         | 10 |
| Diacetone alcohol                                                                             | 5  |
| Water                                                                                         | 1  |

JOHN A. EDGAR.  
HAROLD A. WOODS.

ing 7.0 and the remainder a blend of mineral lubricating oil and a highly aromatic, liquid sulphur dioxide soluble petroleum extract boiling in the kerosene range, said composition having a viscosity of at least approximately 100 S. S. U. at 100° F. and a flash point in excess of 150° F. as determined by the closed cup method A. S. T. M. designation: D93.

2. A flushing oil composition suitable for removing sludge and lacquerous deposits from internal combustion engines comprising the following constituents in the following approximate proportions by weight: